

## [54] METHYLOLPHOSPHORIC TRIAMIDES

[75] Inventor: Patrick Michael Burke, Wilmington, Del.

[73] Assignee: E. I. du Pont de Nemours and Company, Wilmington, Del.

[22] Filed: June 12, 1972

[21] Appl. No.: 261,813

[52] U.S. Cl. .... 260/551 P, 252/8.1, 116/15 F

[51] Int. Cl. .... C07f 9/22

[58] Field of Search ..... 260/551

## [56] References Cited

## UNITED STATES PATENTS

3,711,542 1/1973 Hook et al. .... 260/551

## FOREIGN PATENTS OR APPLICATIONS

1,222,885 2/1971 Great Britain ..... 260/551

## OTHER PUBLICATIONS

Hellmann, Newer Method of Preparative Organic Chemistry, Vol. II, p. 278-79 (Edited by Foerst) (Academic Press, N.Y.) (1963).

*Primary Examiner*—Harry I. Moatz

## [57] ABSTRACT

Methyloolphosphoric triamides, for examples, hexamethyloolphosphoric triamide, useful for rendering combustible cellulosic fabrics flame resistant.

6 Claims, No Drawings

## METHYLOLPHOSPHORIC TRIAMIDES

## BACKGROUND OF THE INVENTION

## 1. Field of the Invention

This invention relates to methylolphosphoric triamides.

## 2. Description of the Prior Art

Phosphorus-containing compounds are well known for their ability to impart flame resistance to fabrics. Compounds which are known for this purpose include tetra(hydroxymethyl)-phosphonium chlorides, aziridinyl phosphine oxides and the methylol amide of the dimethyl ester of bis(carboxyethyl)-phosphonic acid. Many of the prior art compounds may be undesirable as flame retardants for fabrics because they stiffen the fabric, because of their toxicity, because they must be employed in large quantities to impart any significant flame resistance to the fabric, or because they are readily removable by laundering.

German Pat. No. 1,009,629 discloses flame retarding phosphorus compounds which are obtained by treating phosphoric triamide with formaldehyde and methanol. The product, which includes phosphorus esters and hexamethylenetetramine, appears to lack durability to laundering.

British Pat. No. 1,222,885 discloses as flame retardants for cellulosic materials, compounds or combinations of compounds which contain nitrogen and phosphorus. It further discloses that fabrics treated with such a compound or combination of compounds have a good degree of flame resistance if the nitrogen content is equal to or greater than 6 minus 4 times the phosphorus content and, preferably, is at least 2.5 times the phosphorus content, with the preferred amounts of nitrogen and phosphorus totaling at least 3.5 percent, based on the weight of fabric. Exemplary of compounds containing both nitrogen and phosphorus are phosphoric triamides (phosphoramides) having the formula



wherein R is substituted or unsubstituted C<sub>1-6</sub> alkyl, with hydroxyalkyl being a preferred substituted alkyl group.

U.S. Pat. No. 2,661,342 discloses that combustible cellulosic materials can be rendered flame resistant with a resinous aminoplast condensation product in combination with the reaction product of phosphorus oxychloride and ammonia, the reaction product having a nitrogen to phosphorus atomic ratio of 2.1 to 2.3 and a molecular weight of 180 to 300. Aminoplast condensation products are defined therein as resins derived from amino (including imino) or amido (including imido) compounds, a typical example being a urea-formaldehyde resin (Modern Plastics 17, 433, 1939). Other aminoplast resins are described by C. Ellis in "Chemistry of Synthetic Resins," Chapter 26, Reinhold Publishing Co., 1935.

## SUMMARY OF THE INVENTION

It is an object of this invention to provide compositions which are highly effective in imparting flame re-

sistance to combustible cellulosic materials. Another object is to provide phosphorus-containing compositions which impart flame resistance to such cellulosic materials. Still another object is to provide flame resistant cellulosic materials. A further object is to provide such flame resistant materials which are durable to laundering. Still another object is to provide a method for imparting flame resistance to combustible cellulosic materials, which method employs aqueous solutions of phosphorus-containing compounds.

In summary, the present invention resides in the discovery of methylolphosphoric triamides which are useful for imparting flame resistance to combustible cellulosic materials, the triamides having the formula



20

wherein at least one of the six R groups is CH<sub>2</sub>OH and the remainder if any are H, said triamide being characterized by the presence in its P-31 nuclear magnetic resonance (NMR) spectrum of a band in the range 15-20 ppm. downfield from 85 percent aqueous phosphoric acid as external standard. The invention includes the process of applying such triamides to combustible cellulosic materials and, also, the materials which are made flame resistant with such triamides.

## DETAILED DESCRIPTION OF THE INVENTION

This invention is based upon the discovery that the methylolphosphoric triamides as defined above are more effective than prior art compounds of similar structure in imparting flame resistance to combustible cellulosic materials, such as fabrics, and that fabrics can be treated with such methylolphosphoric triamides without substantial alteration of their physical characteristics, such as stiffness or hand. As noted above, the methylolphosphoric triamides of this invention contain one to six methylol substituents (designated as R in the formula). The remaining nitrogen substituents if any (also designated as R in the formula) are hydrogen. In order to simplify the following discussion, the number of methylol groups in the compound of the above formula will be designated as n methylol groups, with n having the value 1 to 6. Correspondingly, the number of hydrogen atoms in the compound of the above formula will be designated 6-n.

The compounds of this invention are all water soluble. As the number n of methylol groups increases, the compounds become more hygroscopic. Analyses of the compounds of this invention by nuclear magnetic resonance show that when the three nitrogen atoms are less than completely substituted with methylol groups, that is, n is less than 6, the compounds are actually mixtures of compounds. It is to be understood, therefore, that the n values reported for such mixtures represent average values, and further, that n need not be a whole number. When the nitrogen atoms are completely substituted with methylol groups (n is 6), the triamide exhibits a single P-31 NMR peak at 16.9 ppm. When n is 1 but less than 6, the triamide exhibits a P-31 NMR peak in the range 15-20 ppm. When n is about 3, there is an unsymmetrical peak at about 18.3 ppm. At higher values of n this peak shifts in its center to a lower reso-

nance value; at lower values of  $n$ , to a higher resonance value.

The compounds of this invention can be prepared by reacting phosphoric triamide and formaldehyde, for example, as a 37 weight percent aqueous solution, in an aqueous medium having a pH of 7-11, preferably 9.5-10.5, obtained by the addition of a base, until the P-31 NMR spectrum of the reaction mixture downfield from 85 percent phosphoric acid as the external standard shows peaks in a band at 15-20 ppm. Preferably, the signal at 22.5 ppm, indicating unreacted phosphoric triamide disappears; normally, this occurs when  $n$  exceeds about 1.5. The reaction proceeds readily at 5°-50°C., preferably at 20°-25°C., and phosphoric triamide readily binds as many as 6 molar equivalents of formaldehyde. Under the preferred conditions the reaction is completed in 1.5-2 hours. The NMR spectrum after 15 minutes exhibits two signals in a band at 15-20 ppm, and after about 90 minutes exhibits a peak in this range, the peak being centered according to the value of  $n$ . The P-31 NMR spectrum provides a ready means of monitoring the reaction. After completion of the reaction, the pH is decreased, for example, by the addition of hydrochloric acid, to 6.5-7.5, preferably to 6.9-7.3. A curing catalyst and/or an aminoplast resin precondensate (both discussed hereinafter) can be added at this stage, either immediately or after the reaction mixture is diluted with water to the desired methylolphosphoric triamide concentration.

Although it is preferred to use the compounds of this invention directly as formed in solution in the reaction mixture, they can be isolated by neutralizing the reaction mixture after completion of the reaction, for example, by adjusting the pH to 7.1-7.5, and the vacuum stripping off the solvent at a solution temperature not in excess of 50°C. The isolated compounds are solids or viscous liquids which can be redissolved in aqueous media, from which the compounds can be applied to the combustible cellulosic material which is to be rendered flame resistant.

The compounds of this invention wherein  $n$  is less than 6 have limited storage stability in aqueous solution. Such aqueous solutions generally should be employed within about 4 hours of preparation in order to impart durable flame resistance. The instability of such aqueous solutions is evident from a study of the P-31 NMR spectrum. Upon aging, the aqueous solution becomes acid, the P-31 NMR spectrum becomes more complex and there may be noted a decrease in the amount of material having peaks in the 15-20 ppm. range. Correspondingly, the flame resistance imparted to combustible cellulosic materials with such aged aqueous solutions is less fast to laundering.

The efficiency, on a weight basis, of the compounds of this invention varies with the value of  $n$ . Combustible cellulosic materials are most efficiently rendered flame resistant by the (mono- to tri-)methylol compounds, less efficiently by the (tetra- to hexa-)methylol compounds. Preferred are the (di- and tri-)methylol compounds. Only slight loss of hand accompanies treatment of fabrics with the (mono- to tri-)methylol compounds while a greater loss of hand accompanies the use of the (tetra- to hexa-)methylol compounds.

The flame resistance imparted to combustible cellulosic materials by the compounds of this invention is made durable to laundering by curing the compounds after they have been applied to the substrates from an

aqueous solution. After application the material is dried by heating at a temperature up to 140°C., preferably at 100°-115°C. Curing is effected by heating the dried material at 150°-190°C., preferably at 160°-170°C., in the presence of an acidic curing catalyst for 2-10 minutes, preferably 2-4 minutes. The catalyst usually is dissolved in the aqueous solution of methylolphosphoric triamide before the latter is applied to the material being treated. The catalyst usually is added to such aqueous solution, such as a padbath, in an amount which is 0.5-5 weight percent, preferably 1-2.5 percent, based on the weight of the solution. Optionally, the drying and curing steps can be carried out at the curing temperature.

In the cured condition, fabrics treated with methylolphosphoric triamides of this invention lose very little flame resistance after the first laundering; fabrics which have been treated with the di- and higher methylol phosphoric triamides retain their flame resistance even after being subjected to multiple launderings. During the curing step, the compounds of this invention are converted to insoluble polymeric materials, thus rendering them durable to laundering. This explanation of durability is not intended as limiting since it is recognized that an entirely different mechanism or a combination of mechanisms may be involved in the fixing operation. For example, it is recognized that durability, in part, may be the result of chemical bonding between the compounds of this invention and the substrate cellulosic material.

Preferred curing catalysts are acids which are relatively nonvolatile at curing temperatures and latent acid compounds. Examples of these include oxalic, glycolic, lactic, malic, tartaric, succinic and citric acids, ammonium chloride, ammonium sulfates, ammonium phosphates, such as diammonium acid phosphate, acid salts of organic amines, such as 2-methyl-2-aminopropanol-1 hydrochloride and tris(2-hydroxyethyl)amine hydrochloride, and salts of weakly basic metals and strong acids, such as zinc nitrate, zinc chloride, zinc fluoborate, magnesium chloride and magnesium nitrate.

The compounds of this invention impart flame resistance to combustible cellulosic materials by their application to or incorporation into the material in amounts of 10-60 weight percent, based on the dry weight of the material being treated. Generally, the amount added is 14-50 percent, preferably 14-25 percent. The compounds can be applied or incorporated in any suitable fashion. Conveniently, they are applied as 5-65 weight percent aqueous solutions by a padding operation; preferably, the aqueous solution contains 15-50 percent of a methylolphosphoric triamide of this invention.

The aqueous solution of methylolphosphoric triamide can contain wetting agents, for example, non-ionic wetting agents, to facilitate wetting of the cellulosic material being treated. Included among such wetting agents are polyethylene oxides obtained by reacting a phenol or a monohydric or polyhydric aliphatic alcohol with ethylene oxide. Such wetting agents generally are added so as to comprise 0.01-0.15 weight percent of the aqueous triamide solution.

If the aqueous padbath method of application is employed, the padbath, for example, the preparative reactive mixture described above, at a pH of 6.5-7.5, is padded onto the substrate to the extent of 50-120 per-

cent, based on the dry weight of substrate, preferably to the extent of 60-90 percent. Padding can be effected by soaking the fabric in the padbath and squeezing out the excess solution, thus providing control of the net amount of solution applied to or picked up by the fabric. The fractions of the solutions retained by and squeezed out of the fabric are of essentially the same composition. Preferably, the curing catalyst is incorporated into the padbath. Drying and curing are carried out as previously described. Conveniently, continuously circulating hot air can be employed as a heat source, especially for the drying operation.

Instead of padding the solution onto the fabric which is to be treated, other convenient means of application can be employed. For example, the solutions of the compounds of this invention can be sprayed, in controlled amounts, onto moving fabrics.

The compounds of this invention can be employed in combination with well-known aminoplast resin condensates which, in some instances, improve the effectiveness of the compounds of this invention in rendering cellulosic materials flame resistant. It also has been discovered that the aminoplast resins, in some instances, improve the durability of the compounds of this invention when both have been coapplied to the substrate. Aminoplast resins are well known in the art and have been discussed hereinabove. Many such resins are known to impart flame resistance to cellulosic materials. They often are applied as water soluble precondensate compounds. When such precondensates are employed herein, they are dissolved in the freshly prepared solution of the methylolphosphoric triamide, which solution then is preferably used promptly to treat the fabric, for example, within about 4 hours.

When a methylolphosphoric triamide of this invention is employed in combination with a water soluble aminoplast resin precondensate, less than the previously recited amounts of the triamide are necessary to impart the desired flame resistant characteristics to the cellulosic material being treated. When used in such a combination, the methylolphosphoric triamide is incorporated into or applied to the material in amounts 7-15 weight percent, preferably 8-12 percent, based on the dry weight of material being treated. The amount of aminoplast precondensate added in combination with the trimethylolphosphoric triamide is known from the art. When the aminoplast resin precondensate is a hydroxymethylmelamine, a convenient amount is 7-13 weight percent, based on the dry weight of material being treated, preferably 7-10 percent.

Water soluble aminoplast resin precondensate compounds useful with the compounds of this invention include those containing at least two moles of condensed formaldehyde, as N-hydroxymethyl or N-alkoxymethyl groups wherein the alkoxy group contains 1-4 carbon atoms. Precondensate compounds include polymethylol derivatives, as well as their partial or complete ethers, of amides such as urea, thiourea, guanidine and dicyandiamide, for example, dimethylolurea, tetramethylol urea, di(methoxymethyl)urea, dimethylol-*quani*dine, trimethylol quanidine and dimethylol-dicyandiamide. Precondensate compounds of substituted ureas can also be used, such as formaldehyde condensates, and their ethers, of ethylene urea, methyleneurea, acetylenediurea, biuret, oxydimethyleneurea (uron) and iminodimethyleneurea (triazone). Particular examples of these include dime-

thylolethyleneurea, dimethylolmethyleneurea, tetramethylolacetylenediurea, trimethylolbiuret, di(methoxymethyl)uron and di(methoxymethyl) triazone.

Still other precondensate compounds include the reaction products of formaldehyde and triazines such as melamine, diaminotriazine, formoguanamine and 2-chloro-4,6-diaminotriazine. Preferred examples of such precondensates include di- and trimethylolmelamine, optionally partially methylated, hexa(methoxymethyl)melamine, tetramethyloldiaminotriazine and tetramethylol-2-chloro-4,6-diaminotriazine. Diazines and azoles are also useful aminoplast resin precondensate compounds. Typical of these are precondensates based on 2,4-diamino-1,3-diazine, guanazole and diaminopyrrole.

As previously indicated, fabrics which are treated with the compounds of this invention substantially retain their original physical characteristics, such as softness and hand. Even when the compounds of this invention are employed in combination with aminoplast resin precondensates, because of the small quantity of each compound required, the properties of the fabric are altered only slightly, especially with the preferred aminoplast resin precondensates and the preferred methylolphosphoric triamides.

The compounds of this invention and their combinations with aminoplast resin precondensate compounds are particularly effective on combustible cellulosic materials of a fibrous nature. In the textile field, this includes cotton, the preferred fiber, linen, viscose rayon, cuprammonium rayon, jute, hemp and ramie. Such cellulosic material can be treated in the form of raw fiber, carded stock, rovings, thread, yarn and felts as well as in the form of knitted and woven fabrics. However, the cellulosic material need not be fibrous to be rendered fire resistant with the compounds of this invention; any cellulosic material can be treated if it can be penetrated or swollen by water, thus permitting penetration by the aqueous medium containing the methylolphosphoric triamide. Fibrous cellulosic material can be rendered flame resistant with the compounds of this invention even though it is blended with other fibers, for example, natural animal fibers such as wool and synthetic fibers such as linear polyamide, linear polyester and polyacrylic fibers.

Cellulosic materials which have been rendered flame resistant with the compounds of this invention are especially useful in tents, stage scenery, upholstery fabrics, slipcovers, draperies, wearing apparel for personnel in close contact with fire or heat, bedding, nightclothes, tarpaulins, insulation, padding, rope, string and twine. Fabrics which have been treated with the compounds of this invention are flame resistant throughout, not just on their surfaces.

In the following examples, parts are parts by weight except where otherwise specified. The terms hand, padding, laundering, limiting oxygen index (LOI), vertical flame test (VFT) and char length refer to the following:

Hand: the softness of a treated fabric relative to untreated fabric as the control. It is graded subjectively here on a scale of 1 to 5 in which 5 signifies a softness and flexibility virtually indistinguishable from the control and 1 signifies great stiffness relative to the control

Padding: wetting the fabric with the aqueous triamide solution and then running the wet fabric between rol-

lers to squeeze out liquid which is in excess of the desired pickup on the fabric.

Laundering, also expressed as home washing (HW): exposing the fabric to a standard laundering cycle, employing a washing solution of 100 grams of a commercial detergent ("Tide") per 15 gallons of water, and tumble drying the washed fabric.

Limiting Oxygen Index: determined with a 5-inch by 2-inch piece of fabric spread lengthwise in a vertical plane and supported along its vertical edges. The spread fabric is positioned inside a transparent circular (cylindrical) column open only at the top. The top of the column is one or more inches above the spread fabric. The interior of the column is provided with an upward flow, from its base, of a gaseous mixture of pure oxygen and pure nitrogen. The volume flow rate of each gas making up the mixture is instrumented and manually adjustable. To test fabric in this apparatus, the spread fabric is ignited from the top while gas mixture flows up the column. The flow rates of the nitrogen and oxygen are adjusted until the flame on the ignited fabric just goes out. The ratio of the volume flow of oxygen to the sum of the volume flows of oxygen and nitrogen is then calculated. This value, called the Limiting Oxygen Index or LOI, is the average of two determinations. As a standard of reference, untreated 8-oz. cotton twill used in the following examples to test the effectiveness of the compounds of this invention has an LOI value of  $0.180 \pm 0.002$  and is completely burned up in the vertical flame test. Air contains about 21 mole percent oxygen; therefore, fabrics with LOI values below about 0.210 can be expected to burn freely in a candlelike manner (from the top to the bottom) in air. For commercial applications, an LOI value of at least about 0.260-0.270 is considered acceptable.

Vertical Flame Test and Char Length: carried out in a 12-inch by 12-inch cabinet 30 inches high and having a glass front. Gas circulation is provided by a 4-inch high opening beneath the glass front and a 6-inch diameter baffled hole at the top of the cabinet. It is provided with holder brackets on which a specimen holder is hung. The specimen holder provides a 2-inch wide by 14-inch high vertical open space and vertical side clips to hold edges of fabric which span this open space. Samples are ignited by a 6-inch high Bunsen burner having a 0.375-inch inside diameter tube and a luminous flame 1.5 inches long. To conduct the test, a 2.75-inch by 10-inch fabric sample is held in the specimen holder by its vertical edges and the specimen holder is hung centrally by the holder brackets. The igniting flame is applied so that 0.75 inch of the lower end of the fabric is in the flame. This exposure is continued for 3.0 seconds and the flame is removed. After the flame has extinguished itself, the sample is removed from the holder. A hook with an attached weight is inserted into the sample on one side of the charred area 0.25 inch from the outside edge and 0.25 inch from the lower edge. For 2.0 to 6.0-oz. per square yard fabric, the attached weight is 0.25 pound; for over 6.0 and up to and including 15-oz. per square yard fabric, a 0.50 pound weight is used. The corner of the cloth at the opposite edge of the char from the load is gently raised until the sample and weight are clear of supporting surface. The length of the tear which occurs is measured (in inches) and reported as char length. Where char length is reported below, it is understood to have been determined

by this procedure and to be an average value of 2 or 4 determinations.

#### EXAMPLE 1

- 5 Trimethylolphosphoric Triamide Preparation  
 9.5 Parts (0.1 mole) of phosphoric triamide, prepared according to Klement and Koch, Berichte 87, 338 (1954) and 25 parts of 37 percent aqueous formaldehyde (0.3 mole) were mixed at 20°C. and the pH of  
 10 the resulting solution was adjusted to 10.3 with 20 percent aqueous sodium hydroxide. The solution was allowed to stand for 2.5 hours, after which time the pH of the solution had dropped to 9.9 and the P-31 NMR spectrum showed a band between 15 and 20 ppm. with  
 15 an unsymmetrical peak centered at 18.3 ppm.; the spectrum was free of a signal at 22.5 ppm. The pH of the solution was then adjusted to 7.6 with 10 percent hydrochloric acid. Water was rapidly stripped from the solution at 20 mm. of Hg pressure and 50°C. (using a  
 20 Rotovac still). 20.2 Parts of residue (theoretical: 18.5 parts) were obtained as an extremely viscous mass which, on standing, became a soft transparent solid. This solid was chemically analyzed. Calc'd for  $C_3H_{12}O_4N_3P$ : C, 19.5; H, 6.5; N, 22.7; P, 16.8; Atomic  
 25 N/P ratio, 3.0. Found: C, 19.8; H, 6.6; N, 21.1; P, 15.9; Atomic N/P ratio, 2.9.

#### EXAMPLE 2

- 30 Hexamethylolphosphoric Triamide Preparation  
 0.1 Mole of phosphoric triamide and 0.72 mole of formaldehyde (37 percent aqueous solution) were reacted at a pH of 10.2 as described in Example 1. There was no drop in pH of the solution after standing. The product in solution showed a single P-31 NMR peak  
 35 versus 85 percent phosphoric acid at 16.9 ppm. Adjustment of the pH to 7.6 with 10 percent hydrochloric acid followed by stripping of water at 50°C. and 20 mm. of Hg pressure provided 32.0 parts (theoretical: 27.5 parts) of a colorless viscous liquid residue which was  
 40 analyzed by chemical analysis. Calc'd for  $C_6H_{18}O_7N_3P$ : C, 26.2; H, 6.6; N, 15.3; P, 11.3. Found: C, 33.5; H, 7.6; N, 13.0; P, 9.6. Since the 37 percent aqueous formaldehyde solution employed in this experiment had been stabilized with 10-15 percent methanol, it is believed that etherification of the methylol groups may have occurred during stripping. The P-31 NMR spectrum of the product redissolved in water showed peaks at 16.9 ppm. (for the hexaformaldehyde adduct) and at 11.3 ppm. (believed to correspond to methoxymethyl derivatives of phosphoric triamide). The analytical results confirm the presence of almost three methoxy groups in the product (replacing almost three hydroxy groups of the hexamethylolphosphoric triamide).  
 45 Calc'd. for  $C_9H_{24}O_7N_3P$ : C, 34.0; H, 7.6; N, 13.2; P, 9.8.  
 50

#### EXAMPLE 3

##### Methylolphosphoric Triamide/Trimethylolmelamine Treatment of Cotton Fabric

- 60 Seven padbaths were prepared so as to contain equal amounts of phosphoric triamide (PTA), 0.5 weight percent ammonium chloride (curing agent) and trimethylolmelamine (TMM) in an amount 1.67 times the PTA. To six of the baths were added 1, 2, 3, 4, 5 and 6 molar equivalents, respectively, of formaldehyde, as a 37 percent aqueous solution. The formaldehyde and PTA were allowed to react at a pH of 10° at 20°C. for 2 hours, after which the pH was adjusted to 7.5.

Eight-ounce cotton twill fabrics were impregnated in the padbaths and squeezed to a net pickup on the fabrics approximating 6.6% PTA and 11.0% TMM. The fabrics were heated at 100°C. until dry to the touch and then cured at 170°C. for 4 minutes. They were chemically analyzed as cured, tested for LOI, laundered once (one home wash) and rate for hand, laundered 19 more times (total, 20 home washes) and then chemically analyzed and tested for LOI. The results are summarized in the following table.

## EXAMPLE 4

## Trimethylolphosphoric Triamide Treatment of Cotton Fabric

A solution of trimethylolphosphoric triamide was prepared as in Example 1. Eight portions, neutralized to pH 7.0, were diluted with water to provide concentrations of 4-32 percent as shown in the following table. 0.5 Weight percent 2-methyl-2-aminopropanol-1 hydrochloride (curing agent), based on the bath 10 weight, was added to each bath. These baths were pad-

| Analysis<br>After Cure          | Mole Ratio CH <sub>2</sub> O/PTA |       |       |       |       |       |       |
|---------------------------------|----------------------------------|-------|-------|-------|-------|-------|-------|
|                                 | 0                                | 1     | 2     | 3     | 4     | 5     | 6     |
| % P                             | 2.03                             | 1.84  | 1.81  | 1.84  | 1.90  | 1.84  | 2.01  |
| % N                             | 6.46                             | 5.96  | 6.40  | 6.39  | 6.29  | 6.34  | 6.52  |
| % PTA (on<br>wt. of<br>fiber)   | 7.3                              | 6.6   | 6.6   | 6.6   | 6.8   | 6.6   | 7.2   |
| % Methylol<br>Compound          | —                                | 8.7   | 11.8  | 12.9  | 15.4  | 17    | 20.9  |
| % TMM                           | 12.2                             | 11.0  | 11.0  | 11.0  | 11.3  | 11.0  | 12.0  |
| <u>LOI</u>                      |                                  |       |       |       |       |       |       |
| As Cured                        | 0.444                            | 0.377 | 0.356 | 0.331 | 0.324 | 0.316 | 0.302 |
| After 1 Home<br>Wash            | 0.308                            | 0.352 | 0.372 | 0.342 | 0.318 | 0.326 | 0.305 |
| After 20<br>Home Washes         | 0.223                            | 0.341 | 0.375 | 0.348 | 0.333 | 0.334 | 0.312 |
| <u>After 20<br/>Home Washes</u> |                                  |       |       |       |       |       |       |
| % P                             | 0.99                             | 1.28  | 1.60  | 1.98  | 1.64  | 1.82  | 1.82  |
| % N                             | 1.51                             | 4.69  | 5.81  | 6.11  | 5.99  | 6.45  | 6.25  |
| % of Initial<br>P Retained      | 49                               | 70    | 88    | 107   | 86    | 99    | 91    |
| Hand after<br>1 Home Wash       | 5                                | 4-5   | 4     | 4     | 4-3   | 3     | 2     |

These results show the superiority of methylolphosphoric triamide/trimethylolmelamine compositions over phosphoric triamide/trimethylolmelamine compositions for imparting flame resistance. Further, they show that the flame resistance imparted by the di- and higher formaldehyde adducts improves with launderings. They also demonstrate the minimal loss of hand in cellulosic fabrics treated with the compositions containing (mono- to tri-)methylolphosphoric triamides.

ded onto 8-oz. cotton twill fabric samples to net solution pickups of about 87 percent. The padded fabrics were dried at 115°C. and then cured for 4 minutes at 165°C. The cured fabrics were laundered 20 times. Elemental chemical analyses of the fabric samples as cured (before laundering) and after 20 launderings were made. LOI tests for flame resistance were made as cured, after one laundering and after 20 launderings. 45 50 The following table summarizes the results.

| % Trimethylol<br>PTA in Bath | % Trimethylol PTA<br>(on weight of fiber) |                                 |       | LOI     |       |       | % P Re-<br>tained<br>(20 HW) | Atomic Ratio N/P<br>Initial | Atomic Ratio N/P<br>20 HW |  |  |  |
|------------------------------|-------------------------------------------|---------------------------------|-------|---------|-------|-------|------------------------------|-----------------------------|---------------------------|--|--|--|
|                              | Calc'd                                    | Found<br>(from P,N<br>analyses) |       | Initial | 1 HW  | 20 HW |                              |                             |                           |  |  |  |
|                              |                                           |                                 |       |         |       |       |                              |                             |                           |  |  |  |
| 4                            | 3.5                                       | 3.4                             | 0.201 | 0.203   | 0.189 | 59    | 2.9                          | 2.7                         |                           |  |  |  |
| 8                            | 7.0                                       | 6.4                             | 0.237 | 0.224   | 0.215 | 71    | 3.0                          | 2.7                         |                           |  |  |  |
| 12                           | 10.5                                      | 10.2                            | 0.257 | 0.243   | 0.245 | 83    | 2.8                          | 2.7                         |                           |  |  |  |
| 16                           | 14.0                                      | 13.6                            | 0.273 | 0.263   | 0.264 | 75    | 2.8                          | 2.8                         |                           |  |  |  |
| 20                           | 17.5                                      | 16.2                            | 0.287 | 0.278   | —     | 87    | 3.0                          | 2.8                         |                           |  |  |  |
| 24                           | 21.0                                      | 19.5                            | 0.292 | 0.290   | 0.328 | 88    | 3.0                          | 2.8                         |                           |  |  |  |
| 28                           | 24.5                                      | 24.2                            | 0.298 | 0.297   | 0.313 | 91    | 3.0                          | 2.8                         |                           |  |  |  |
| 32                           | 28.0                                      | 26.1                            | 0.293 | 0.300   | 0.318 | 92    | 3.1                          | 2.9                         |                           |  |  |  |

These results show the efficiency of trimethylolphosphoric triamide in imparting flame resistance to cotton fabric and the durability of that effect even after repeated laundering.

## EXAMPLE 5

## Dimethylolphosphoric Triamide/Trimethylolmelamine Treatment of Cotton Blend Fabrics

Dimethylolphosphoric triamide was prepared in solution from phosphoric triamide (PTA) according to the procedure of Example 1 except that 16.7 parts, instead of 25 parts, of aqueous formaldehyde were employed. Six padbaths were prepared from the solution, each neutralized to pH 7.2 and containing trimethylolmelamine (TMM) and 0.5 weight percent of ammonium chloride (curing agent). The padbaths were padded onto commercial lightweight, 2.8-oz. and 5.3-oz. 50/50 polyester/cotton and 3.6-oz. 50/50 rayon/cotton blend fabrics, the fabrics were dried, and curing was carried out in a manner similar to the procedures previously described. The following table summarizes the results of the evaluations of the treated fabrics.

| Fabric                   | Wt. % Dimethylol PTA<br>(on weight of fiber) | Wt.%<br>TMM | LOI     |       |       |      |
|--------------------------|----------------------------------------------|-------------|---------|-------|-------|------|
|                          |                                              |             | Initial | 1 HW  | 20 HW | Hand |
| 2.8 oz. polyester/cotton | 11.3                                         | 7.0         | 0.236   | 0.237 | 0.234 | 4    |
| 2.8 oz. polyester/cotton | 18.3                                         | 7.0         | 0.244   | 0.247 | 0.245 | 3-4  |
| 5.3 oz. polyester/cotton | 13.1                                         | 7.7         | 0.251   | 0.249 | 0.244 | 3    |
| 5.3 oz. polyester/cotton | 21.6                                         | 7.7         | 0.257   | 0.259 | 0.259 | 2    |
| 3.6 oz. rayon/cotton     | 9.6                                          | 8.0         | 0.276   | 0.276 | 0.284 | 4    |
| 3.6 oz. rayon/cotton     | 16.6                                         | 8.0         | 0.277   | 0.294 | 0.300 | 3-4  |

## EXAMPLE 6

## Trimethylolphosphoric Triamide Treatment of Cotton Fabrics

This example shows the beneficial effect that can be realized through use of the combination of trimethylolphosphoric triamide and trimethylolmelamine (TMM) in imparting flame resistance to fabrics. The trimethylolphosphoric triamide was prepared from phosphoric triamide according to the procedure described in Example 1. Padbaths were prepared in a manner similar to that described in Example 5. The impregnated fabrics (8-ounce cotton twill fabric) were dried at 115°C., cured at 165°-175°C. and given one home wash. The following table summarizes the results of the evaluations of the treated fabrics.

| Wt. % Additive on Fabric |     |       |
|--------------------------|-----|-------|
| Trimethylol PTA          | TMM | LOI   |
| 0                        | 8   | 0.189 |
| 0                        | 16  | 0.195 |

The padbaths were padded (at 87 percent add-on) unto mercerized bleached cotton twill 8-oz fabrics (also designated A through F to correspond to padbaths A through F). The padded fabrics were dried at 100°C. for 10 minutes, then cured at 165°C. for 4 minutes. The following table summarizes the results of the evaluations of the treated fabrics.

| LOI                     | A     | B     | C     | D     | E     | F     |
|-------------------------|-------|-------|-------|-------|-------|-------|
| Initial                 | 0.251 | 0.295 | 0.263 | 0.244 | 0.261 | 0.233 |
| After 1 home wash       | 0.245 | 0.296 | 0.270 | 0.250 | 0.254 | 0.239 |
| After 20 home washes    | 0.229 | 0.302 | 0.276 | 0.248 | 0.206 | 0.233 |
| VFT (in inches)         |       |       |       |       |       |       |
| Initial                 | 4.8   | 0.75  | 1.4   | 4.1   | 2.4   | 4.0   |
| After 20 home washes    | BEL   | 1.3   | 0.6   | 4.5   | BEL   | 3.3   |
| Wt. % P on Fabric       |       |       |       |       |       |       |
| Initial                 | 1.41  | 1.35  | 1.36  | 1.35  | 1.28  | 1.31  |
| % of Initial P Retained |       |       |       |       |       |       |
| After 20 home washes    | 60    | 87    | 70    | 85    | 49    | 88    |

| Wt. % Additive on Fabric |     |       |
|--------------------------|-----|-------|
| Trimethylol PTA          | TMM | LOI   |
| 0                        | 20  | 0.204 |
| 3.4                      | 0   | 0.203 |
| 6.4                      | 0   | 0.224 |
| 8.7                      | 7   | 0.293 |
| 10.2                     | 0   | 0.243 |
| 19.5                     | 0   | 0.290 |
| 24.2                     | 0   | 0.297 |

## EXAMPLE 7

## Trimethylolphosphoric Triamide/Aminoplast Resin Treatment of Cotton Fabric

Six aqueous padbaths (designated A through F) were prepared so as to contain, per 100 parts of solution, 12 parts of trimethylolphosphoric triamide, 1 part of 2-methyl-2-aminopropanol-1 hydrochloride (curing agent) and a water soluble aminoplast resin precondensate. Shown in the following table are the precondensates and the amounts which were added (along with the triamide and curing agent) to the padbaths to provide equivalent nitrogen contents.

The embodiments of the invention in which an exclusive property or privilege is claimed are defined as follows:

1. Methylolphosphoric triamide having the formula



wherein at least one of the six R groups is  $\text{CH}_2\text{OH}$  and the remainder if any are H, said triamide being characterized by the presence in its P-31 nuclear magnetic resonance spectrum of a band in the range 15-20 ppm. downfield from 85 percent aqueous phosphoric acid as external standard.

2. The triamide of claim 1 wherein the number of  $\text{CH}_2\text{OH}$  groups is 2-3 and the P-31 spectrum is free of a band at 22.5 ppm.

3. The triamide of claim 2 wherein the number of  $\text{CH}_2\text{OH}$  groups is three.

4. Process for preparing a methylolphosphoric triamide having the formula

5



wherein 1-5 of the six R groups are  $\text{CH}_2\text{OH}$  and the remainder are H, said triamide being characterized by the presence in its P-31 nuclear magnetic resonance spectrum of a band in the range 15-20 ppm. downfield from 85 percent aqueous phosphoric acid as external standard, which process comprises reacting phosphoric triamide and at least one molar equivalent of formaldehyde in an aqueous medium at a pH of 7-11 until the reaction mixture shows said band in its nuclear magnetic resonance spectrum.

5. The process of claim 4 wherein 2-3 molar equivalents of formaldehyde are reacted with the phosphoric triamide.

6. The process of claim 4 wherein the reaction is carried out at a pH of 9.5-10.5.

\* \* \* \* \*

25

30

35

40

45

50

55

60

65